

(No Model.)

E. P. THOMPSON.

PROCESS OF MAKING INCANDESCENTS.

No. 366,353.

Patented July 12, 1887.



Witnesses

Geo. W. Greek  
Carrie E. Ashby

By his Attorneys

Inventor

E. P. Thompson  
Pope Edgecomb

# UNITED STATES PATENT OFFICE.

EDWARD P. THOMPSON, OF ELIZABETH, NEW JERSEY.

## PROCESS OF MAKING INCANDESCENTS.

SPECIFICATION forming part of Letters Patent No. 366,353, dated July 12, 1887.

Application filed September 15, 1886. Serial No. 213,577. (No model.)

*To all whom it may concern:*

Be it known that I, EDWARD P. THOMPSON, a citizen of the United States, residing in Elizabeth, in the county of Union and State

5 of New Jersey, have invented certain new and useful Improvements in the Process of Forming Incandescent Electric-Light Filaments, of which the following is a specification.

The invention relates to the process of depositing carbon upon electric-light filaments.

The invention consists, in general terms, in applying a hydrocarbon vapor under pressure to a filament while a current of electricity is being passed through the same, the object being to cause the hydrocarbon to permeate the filament, thus filling the pores instead of being deposited merely upon the surface.

The accompanying drawing illustrates an apparatus adapted to carry out the invention.

20 Referring to the figure, A represents a bell-jar adapted to be placed upon a stand or table, B, and fit tightly against the same in any usual manner. A suitable clamp, c, and binding-screw c' may be employed in holding the jar

25 in position. A tube, c'', leads from the bell-jar and is provided with a valve, c', for allowing the air to be expelled therefrom. It is designed that a filament, D, shall be placed within the globe, being held by suitable clamps,

30 d' d'', which are connected with the respective poles of a generator, E, by conductors 1 and 2, the latter of which may include a galvanometer, F. A tube, g, leads from a tank or vessel, G, to the bell-jar. This tube is em- 35 ployed for conducting hydrocarbon vapor from the vessel or tank G to the bell-jar. Preferably the tube is covered with asbestos or other heat-retaining substance for the purpose of preventing the carbon vapor from losing

40 its heat. The tank containing the hydrocarbon liquid is maintained at a temperature sufficient to vaporize the same by means of a furnace or lamp, as shown at H. By means of the heat the vapor may be placed under enor-

mous pressure. A safety-valve, h, may be applied to the tank for the purpose of preventing too great a pressure on the part of the vapor.

In practice the filament is raised to a high temperature by means of an electric current 50 caused to traverse a circuit including the filament. At the same time hydrocarbon vapor is caused to fill the bell-jar, and, being under pressure, it is forced into the pores of the filament, which are opened by reason of the heat. 55 The galvanometer F serves to indicate the strength of current being employed, and also by means of its position it may be determined when the filament has obtained the required thickness and density.

60 I claim as my invention—

1. The combination, substantially as hereinbefore set forth, of a jar for receiving an incandescent electric-light filament, means for placing the filament in an electric circuit, a 65 source of hydrocarbon vapor, and means for causing said vapor to be held in the jar under pressure.

2. The hereinbefore described process of treating filaments for incandescent electric 70 lights, which consists in applying a hydrocarbon vapor to the same under pressure, and at the same time heating the filaments by an electric current.

3. The combination, with a bell-jar and 75 means for inclosing an incandescent electric-light filament within the same, of an electric circuit, including the filament, of a vapor supply, an escape-valve, and means for maintaining the vapor within the jar under pressure.

In testimony whereof I have hereunto subscribed my name this 17th day of August, A. D. 1886.

EDWARD P. THOMPSON.

Witnesses:

DANL. W. EDGECOMB,  
CHARLES A. TERRY.